

# UNITED STATES PATENT OFFICE.

HERMANN GUTZKOW AND BENNO HOMOLKA, OF FRANKFORT-ON-THE-MAIN, GERMANY, ASSIGNORS TO THE FARBWERKE, VORMALS MEISTER, LUCIUS & BRÜNING, OF HÖCHST-ON-THE-MAIN, GERMANY.

## PROCESS OF DYEING COAL-TAR COLORS.

SPECIFICATION forming part of Letters Patent No. 663,225, dated December 4, 1900.

Original application filed February 15, 1900, Serial No. 5,300. Divided and this application filed September 25, 1900. Serial No. 31,086. (No specimens.)

*To all whom it may concern:*

Be it known that we, HERMANN GUTZKOW, chemist, a citizen of the Empire of Germany, and BENNO HOMOLKA, Ph. D., a citizen of the Empire of Austria-Hungary, both residing at Frankfort-on-the-Main, Germany, have invented new and useful Improvements in Producing on the Fiber Dyes Fast to Washing and Acids, of which the following is a specification.

We have shown in our American application, Serial No. 5,300, of February 15, 1900, that a long series of coal-tar colors containing in their molecule once or more the primary or secondary amido or hydroxyl group may be transformed into new products if these colors be treated under certain conditions with such aromatic bases as contain in the molecule once or more the bivalent group  $-\text{NH}-\text{CH}_2-$  or  $-\text{NR}-\text{CH}_2-$  (wherein "R" means alkyl) linked on both sides to benzene, (toluene or xylene.) We have further found that by means of this peculiar chemical process remarkable shades fast to washing and acid may be obtained on the fiber, and this in such a manner that the textile fabric dyed with the above-named coal-tar colors be subsequently treated with the said aromatic bases in form of their salts soluble in water.

The practical application of our process consists in introducing the textile fabric dyed with the above specified coal-tar colors into a dilute aqueous solution of a salt of one of the above-named bases for a short time at a high temperature or for a longer time at indoor temperature till certain signs permit to judge of the completion of the reaction. The goods are then taken out of the bath, rinsed with water, and further worked in the usual manner.

The following examples may illustrate our process:

*Example I—Benzalviolet, (Döbner's violet.)*—Cotton dyed with benzalviolet in the usual manner is introduced into the solution of the hydrochlorid of ortho-amido-metaxylyl-para-toluidin, thirty-two parts of the dyestuff employed being taken for fifty parts of the salt. The whole is then heated at from

60° to 70° till the known violet color becomes 50 green-blue. The goods are then rinsed with water and finished in the usual manner.

*Example II—Fuchsin.*—The process here is the same as in Example I, a deep violet of great fastness to washing being obtained. 55

*Example III—Congo colors.*—As Congo dyestuffs we understand here those substantive cotton dyestuffs as are obtained or supposed to be obtained by the action of tetrazodiphenyl, tetrazoditolyl and similar tetrazo 60 compounds with two nuclei upon aromatic amins, polyaminins, phenols, polyphenols, and amidophenols of the analin and naphthalene series, as well as their sulfonic and carboxylic acids. 65

*Example 1—Congo red.*—Cotton dyed in the usual manner with Congo red is introduced in a wetted state into a bath containing a solution of the hydrochlorid of mono-methyl-para-amidobenzylalcohol obtained 70 by the action of formaldehyde upon the hydrochlorid of monomethylanilin, (0.3 kilograms of the hydrochlorid to fifteen kilograms of dyed goods.) Care must be taken for the bath to react slightly acid on Congo paper, 75 which, if need be, is obtained by carefully adding dilute hydrochloric acid. In this bath the goods assume at once a dark-brown color. The bath is then raised to the boil and maintained at it for about thirty minutes, when 80 the cotton assumes a brownish color. The goods are then taken out, wrung, and washed with a very dilute cold solution of sodium carbonate and finished in the usual manner. The goods are now dyed red, hardly differing 85 in shade from the original one dyed with Congo red, yet absolutely fast to water and scarcely susceptible to dilute acetic acid.

Under certain conditions the transformation of the dyestuff may also be carried out on the 90 fiber in the bath itself after having exhausted it of the greater part of the dyestuff. In this case the bath is slightly acidified by the addition of hydrochloric acid. Then the hydrochlorid of the base is added and the whole is 95 manipulated for another half-hour. The formation on the fiber of the new dyestuffs may also be effected by impregnating and steam-

ing the previously-dyed goods with the solution of the hydrochlorid in question. Instead of the hydrochlorid the salts of all acids preventing the separation of the bases may be employed in this and all other cases.

*Example 2—Benzopurpurin 4 B.*—In this case the process is the same as in the preceding example. The goods are introduced into a solution of the hydrochlorid of the bases, 10 obtained by the reciprocal action of molecular quantities of xylidin, formaldehyde, and hydrochloric acid. It being quite immaterial which xylidin is chosen it is best to use the technical xylidin, being, as is known, a mixture 15 chiefly of asmeta-xylidin, para-xylidin, and small quantities of other xylidins, to fifteen kilograms of cotton, 0.26 kilograms of the base, when the red color becomes at once a deep dark brown. The whole is heated for 20 half an hour at water-bath or even boiling temperature, when the shade of the goods brightens, but only to become red again. The goods are finished according to Example I. 25 The shade thus obtained is of a decidedly-bluer tint than the original benzopurpurin shade, also thoroughly fast to water, not altered by acetic acid, and assuming on addition of dilute hydrochloric acid a brownish color, while the original benzopurpurin on adding 30 dilute mineral acids becomes black-blue and on adding dilute acetic acid dark brown.

*Example 3—Diamin-scarlet 3 B.*—The cotton goods dyed in the usual manner with diamin-scarlet 3 B are introduced into a bath 35 containing a solution of a salt—for instance, the hydrochlorid of the above-mentioned anhydro para-amido-meta-tolylalcohol, when, for instance, fifteen kilograms of the dyed goods are treated with 0.2 kilograms of the 40 said base dissolved in hydrochloric acid. The bath is then heated to from 60° to 70°, when the goods become first dark and finally red. This being done, the goods are taken 45 out, rinsed with water, and finished in the usual manner. The dye thus obtained is of a vivid red, more beautiful and clearer than the original diamin-red dye, while being thoroughly fast to water and boiling acids and indifferent to acetic acid. Under these 50 circumstances the transformation into dyestuffs fast to acid may also be carried out in the

dye-bath itself. In this case the bath is acidified after the greater part of the diamin-scarlet is exhausted. Then the solution of the base is added and the formation of the dyestuff completed by boiling for half an hour. 55 Instead of hydrochloric acid other acids preventing the separation of the base may be used. The formation of the dyestuff may also be effected by way of padding instead of 60 dyeing the dyed goods with the solution of the base and subsequent steaming.

*Example IV—Fluorescein dyestuffs.*—The process here is the same as in the above examples. The dye obtained is considerably 65 bluer than the original eosin-dye and surpasses the latter greatly in fastness to water and acid. The proportional weights of dyestuffs and base in the above examples must not be considered as binding and unalterable. 70 On the contrary, they may be changed within fairly wide limits, according to the effect desired.

We have tested, in a similar way, a long series of coal-tar colors as to their behavior toward the bases mentioned at the beginning. 75 In every case the above-cited fact was confirmed that the choice of the transforming base is quite immaterial upon the result obtained—that is to say, the results obtained so with one and the same dyestuff and different bases do not differ much from each other.

Having now described our process, what we claim is—

The herein-described process for producing 85 on the fiber dyes fast to washing and acids, which consists, in treating textile fabrics dyed with coal-tar colors in the usual manner, with the salts soluble in water of such aromatic bases as contain at least once the bivalent group —NH—CH<sub>2</sub>— linked on both sides to aromatic carbon atoms, substantially as set forth.

In testimony that we claim the foregoing as our invention we have signed our names in 95 presence of two subscribing witnesses.

HERMANN GUTZKOW.  
BENNO HOMOLKA.

Witnesses:

ALFRED BRISBOIS,  
JOHANN HARTEUSTÉR.